# EUROPEAN PATENT SPECIFICATION

(11) **EP 1 013 351 B1**
(45) Date of publication and mention of the grant of the patent: **19.05.2004**
(21) Application number: 99310136.9
(22) Date of filing: 16.12.1999
(51) Int. Cl.: B21B 1/22, C21D 8/02

(54) **Temper rolling method for steel plate and temper rolling mill**
Kaltnachwalzverfahren für Stahlblech und Kaltnachwalzwerk
Procédé d'écrouissage à froid pour tôles d'acier et laminoir d'écrouissage

(30) Priority: 25.12.1998 JP 37029898
(43) Date of publication of application: 28.06.2000
(73) Proprietor: JFE Steel Corporation, Tokyo (JP)
(72) Inventor: Saito, Teruhiro, c/o Chiba Works, Chiba-shi, Chiba 260-0835 (JP); Miyake, Hidenori, c/o Chiba Works, Chiba-shi, Chiba 260-0835 (JP); Kawaguchi, Goro, c/o Chiba Works, Chiba-shi, Chiba 260-0835 (JP); Sato, Naoya, c/o Chiba Works, Chiba-shi, Chiba 260-0835 (JP); Kobayashi, Makoto, c/o Chiba Works, Chiba-shi, Chiba 260-0835 (JP)
(74) Representative: Overbury, Richard Douglas

(56) References cited:
- EP-A- 0 046 423
- EP-A- 0 539 962
- EP-A- 0 679 451
- EP-A- 0 691 412

## Description

The present invention relates to a temper rolling method for steel plate and a to temper rolling mill according to the preambles of claim 1 and claim 6 respectively (see e.g. FR-A 00 46 423). The present invention especially relates to a temper rolling method for a steel plate suitable for producing a can having a highly bright appearance, and to a temper rolling mill for carrying out the method.

Temper rolling of a steel plate requiring brightness before or after plating (for example, a steel plate for producing a can) is usually effected by a dry rolling method using a rolling mill with two stands or more, each stand being allotted a different role. For example, the first stand mainly serves for adjusting the quality of the material (surface hardness and the like) and requires a dull roll having a strong grip force in order to ensure sufficient elongation. This dull roll is usually a roll that has been marked by dull stripes with weakly directional (or generally strongly random) surface roughness produced by shot blasting, electro-spark machining or laser processing. The surface roughness (Ra) is usually 0.5 µm or more.

A grinding processing roll, on the other hand, comprises a so-called mirror bright roll for forming a specular surface appearance, and a so-called scratch bright roll for leaving grinding traces (with a surface roughness (Ra) of about 0.15 µm or more) behind. Some of the scratch bright rolls leave a surface roughness (Ra) of 0.5 µm or more. However, the scratch bright roll is not used in the first stand, since it has been considered to be insufficient for ensuring sufficient elongation.

Conventionally, the steel plate is rolled with the scratch bright roll in the second stand of the rolling mill and thereafter for improving the brightness by alleviating the effect of the dull stripes formed in the preceding stand. The steel plate is then rolled with the scratch bright roll, a mirror bright roll or a dull roll having a surface roughness corresponding to the required surface roughness of the steel plate.

While brightness is improved as the number of scratch bright rolls in the intermediate stands is increased, the facility costs and running costs are increased and a larger installation space is required.

A two stand operation is most advantageous with respect to the production cost. As disclosed in Japanese Unexamined Patent Publication No. 1-95803, a dull roll such as a shot blasted dull roll is used for the front stand and a bright roll is used for the final stand.

The brightness level required with a limited surface roughness has increased in recent years. However, it has been difficult to comply with the requirement of high brightness in temper rolling mills having a small number of stands such as two stand mills, because the number of rollings with the bright roll is decreased in such mills.

While it may be contemplated to apply the rolling mill twice without increasing the number of stands by using the second stand as a pre-stand bright roll, cost increases due to the increased number of steps can not be avoided.

Accordingly, it is therefore desirable to provide a method for improving brightness without incurring additional facilities and production steps.

In one aspect, the present invention provides a temper rolling method for temper rolling a steel plate using a temper rolling mill provided with a plurality of roll stands, wherein at least the roll at the top front stand is a scratch bright roll having a surface roughness (Ra) of 1.2 µm or less, and at least the roll at the last stand is a bright roll having a surface roughness (Ra) of 0.5 µm or less, and wherein the temper rolling is dry rolling and the steel plate contains 0.012 wt% or less of carbon (C). Preferably, the temper rolling mill used in the method has two stands in which case the roll at the first stand is the scratch bright roll having a surface roughness (Ra) of 1.2 µm or less, and the roll at the second stand is the bright roll having a surface roughness (Ra) of 0.5 µm or less.

In another aspect, the present invention provides a temper rolling mill for rolling a steel plate having a plurality of stands, wherein at least the roll at the top front stand is a scratch bright roll having a surface roughness (Ra) of 1.2 µm or less, and wherein at least the roll at the last stand is a bright roll having a surface roughness (Ra) of between 0.15 and 0.3 µm. Preferably, the temper rolling mill is provided with two stands in which case the roll at the first stand is the scratch bright roll having a surface roughness (Ra) of 1.2 µm or less, and the roll at the second stand is the bright roll having a surface roughness (Ra) of between 0.15 and 0.3 µm.

Reference will now be made, by way of example only, to the accompanying drawing, in which:
Fig. 1 is a graph showing the relationship between the carbon (C) content and the elongation of a temper rolled steel plate.

The inventors of the present invention found the following facts through intensive studies:

(A) Brightness is largely deteriorated when a steel plate is compressed using a dull roll having no directional surface roughness such as a shot blasted roll or an electro-spark machined roll at the top front stage of the temper rolling mill.

Brightness, especially brightness after plating, of the steel plate is markedly improved when the steel plate is rolled using a scratch bright roll, even if the surface roughness is comparable to that obtained by other rolling methods. It is conjectured that, since the scratch bright roll leaves unidirectional grinding traces, only a few concave portions called dull bits, which are considered to be a main cause of deterioration of brightness, are formed.

(B) Sufficient elongation cannot be attained when rolling general purpose low carbon steel if a scratch bright roll is used at the top front stand. Although the reason for this is not yet clear, it is conjectured that the surface roughness at the circumference is so weak that the grip force is small since the grinding traces on the surface lie, for example, in radial planes.

On the other hand, in the case of steel plate in which hardness before temper rolling is reduced by reducing the content of carbon (C) to a certain level (so called extremely low carbon steel), an elongation enough for obtaining a desired hardness can be ensured even when a scratch bright roll is used at the top front stand.

The extremely low carbon steel is often excessively elongated when rolled with a dull roll at the top front stand resulting in excess hardness. Or, the elongation may be out of the control limit even though the hardness is not in excess, thereby requiring a quality test to be carried out prior to shipping. On the contrary, when a scratch bright roll is used in place of the dull roll, such excess elongation can be avoided.

The reason why the conditions in the present invention are limited will be described hereinafter.

### [Composition of the target steel plate]

The steel plates to be subjected to the temper rolling method according to the present invention are limited to those containing 0.012 wt% or less of carbon (C), because a desired hardness cannot be attained by elongation using the scratch bright roll at the top front stand when the steel plate contains more than 0.012% of C. More preferably, the steel plate contains 0.0080 wt% or less of carbon. The preferred lower limit for the carbon content is 0.0010 wt%, as lower contents may cause excess elongation.

FIG. 1 shows a graph indicating the relationship between the C content and the elongation of temper rolled steel plate as a result of studies made by the inventors of the present invention. Scratch bright rolls with a surface roughness (Ra) of 0.6 µm, scratch bright rolls with a surface roughness (Ra) of 0.15 µm, and shot blasted dull rolls with a surface roughness (Ra) of 0.6 µm were used as the first stand for obtaining the curves denoted by SB 0.6, SB 0.15 and SB 0.6, respectively, in FIG. 1. Each temper rolling mill comprised two stands, and a scratch bright roll with a surface roughness of 0.2 µm was used at the second stand. An elongation of 1.6% ± 0.2% was obtained with respect to the steel plate containing 0.002 wt% of C under the rolling condition used.

It is apparent from FIG. 1 that elongation of the extremely low carbon steel becomes unstable when the shot blasted dull roll was used at the first stand, (in addition to low brightness). A desired elongation cannot be ensured, on the other hand, when the scratch bright roll with a surface roughness (Ra) of 0.15 µm was used at the first stand. When the scratch bright roll with a surface roughness (Ra) of 0.6 µm was used at the first stand, on the contrary, the desired elongation could be maintained with respect to steel plates with a C content of 0.0012 wt% or less. However, the elongation becomes a little unstable, resulting in a decrease in elongation, in the case of steel plates with a C content of more than 0.0080 wt%.

The steel plate preferably contains either 0.02 wt% of titanium (Ti) or 0.1 wt% of niobium (Nb), or both of them, in order to ensure softness and machinability. Lower limits of 0.005 wt% and 0.002 wt% are recommended with respect to Ti and Nb.

Aluminum (Al) may be present in an amount of 0.15 wt% or less for deoxidation and stabilization of nitrogen (N).

It is preferable to contain other components within the conventional composition range, such as 0.2 wt% or less of silicon (Si), 0.5 wt% or less of manganese (Mn); ( a content of 0.1 wt% or more is more preferable), 0.05 wt% or less of phosphorous (P) and 0.03 wt% or less of sulfur (S). More preferable contents of Si, P and S are 0.05 wt% or less, 0.02 wt% or less and 0.02 wt% or less, respectively.

Calcium (Ca) may be added if desired and the balance is Fe and incidental element and impurities.

### (Roll at the top front stand)

In the front stand at least the top roll is a scratch bright roll with a surface roughness (Ra) of 1.2 µm or less. Brightness before or after plating becomes poor when a dull roll or a scratch bright roll with a surface roughness (Ra) of more than 1.2 µm is used. The preferred lower limit of the surface roughness (Ra) is 0.20 µm or more. When the surface roughness (Ra) is less than 0.20 µm, elongation (hardness) tends to be insufficiently developed. The more preferable surface roughness (Ra) is in the range of 0.5 to 1.0 µm.

Although processing of the rolled surface is not especially limited, chromium (Cr) plating may be effected in view of wear resistance.

### (Roll at the last stand)

According to the method of the present invention, at least the roll at the last stand should be a bright roll with a surface roughness (Ra) of 0.5 µm or less for ensuring a given level or more of brightness. A mirror bright roll or a scratch bright roll may be used depending on the target surface roughness.Nevertheless, a desired brightness (including after plating) cannot be ensured when the surface roughness (Ra) exceeds 0.5 µm. However, the surface roughness is preferably lower than the surface roughness of the roll at the final stand. The effect of the present invention is markedly exhibited using a roll with a surface roughness (Ra) range of about 0.15 to 0.3 µm which is used according to the apparatus of the present invention, where requirements for brightness have not been satisfied using a conventional roll.

Although brightness decreases as the surface roughness of the roll at the top front stand is larger, an improvement in brightness is noticeable by using a scratch bright roll in place of the dull roll at the top front stand even when the rolls have the same surface roughness as each other.

Although the lower limit of the surface roughness as well as the surface treatment after rolling is not especially limited, plating with Cr may be applied to the surface to improve wear resistance.

### (Rolls for the stands other than those described above (three stands or more))

Bright rolls are preferably used for the rolls of the stands intermediate the top front and last stands. A roll having a surface roughness within the range of the surface roughness of the front and last stands is especially suitable for the rolls to be used in the stands other than the front and last stands for ensuring a required brightness. More preferably, the surface roughness of each roll is gradually made finer in the order of from the front roll to the succeeding rolls.

### (Other conditions)

A dry rolling that requires no lubrication of the steel plate is used for the temper rolling. An elongation of 3% or less is suitable, while an elongation of 1.5 ±1% is more preferable and an elongation of 1.5 ±0.5% is further preferable. The target hardness may be 50 to 60 in HR30T.

Plating methods after the temper rolling are not especially designated. Various plating methods generally used for plating steel plates for cans such as tin plating or chromium plating, or nickel (Ni) plating or a chromate processing on the surfaces after these plating treatments may be applied to the target steel plate according to the present invention.

Brightness was measured at an incident light angle of 20° using a gloss meter following JIS Z8741 in the present invention.

The temper rolling mill according to the present invention may be applied to a production line using the temper rolling alone, or it may installed at the outlet of a continuous annealing furnace.

### (Example)

After subjecting the cold roll steel plate having each component shown in TABLE 1 to recrystallization annealing (continuous annealing), the steel plate was temper rolled with a temper rolling mill having two to three sands under the conditions shown in TABLE 2, and the conditions other than those shown in TABLE 2 are the same condition under which an elongation of 1.5 is obtained using the #1 stand SD 0.6 and #2 stand MB 0.5 shown in No. 1 of TABLE 2. After measuring the hardness (HR30T) of each steel plate, it was plated with tin (plating weight of 2.8 g/m²) followed by a measurement of brightness after a reflowing treatment. Brightness was evaluated by the following four steps:
ⓞ: 1300 to 1500
○: 1100 to less than 1300
Δ: 900 to less than 1100
×: less than 900

The results are listed in TABLE 2. It is evident from TABLE 2 that the steel plates obtained according to the present invention had a superior brightness to that of the steel plate in the comparative example.

The present invention enables the production of a steel plate suitable for manufacturing, for example, cans merely by applying unidirectional rolling using a temper rolling mill provided with two to three stands at most.

## Claims

1. A temper rolling method for temper rolling a steel plate using a temper rolling mill provided with a plurality of roll stands, wherein at least the roll at the top front stand is a scratch bright roll having a surface roughness (Ra) of 1.2 µm or less, and at least the roll at the last stand is a bright roll having a surface roughness (Ra) of 0.5 µm or less, **characterised in that** the temper rolling is dry rolling and **in that** the steel plate contains 0.012 wt% or less of C.

2. A temper rolling method according to Claim 1 wherein the temper rolling mill is a two stand mill.

3. A temper rolling method according to Claim 1 or 2 wherein the steel plate contains from 0.001 to 0.008 wt% of carbon.

4. A temper rolling method according to Claim 1, 2 or 3 wherein the steel plate additionally contains from 0.005 to 0.2 wt% of Ti and/or from 0.002 to 0.1 wt% of Nb.

5. A temper rolling method according to any preceding Claim wherein the steel plate additionally contains not more than 0.15 wt% Al, not more than 0.2 wt% Si, 0.1 to 0.5 wt% Mn, not more than 0.05 wt% P, and not more than 0.03 wt% S.

6. A temper rolling mill for steel plate having a plurality of roll stands wherein at least the roll at the top front stand is a scratch bright roll having a surface roughness (Ra) of 1.2 µm or less, **characterised in that** at least the roll at the last stand is a bright roll having a surface roughness (Ra) of between 0.15 and 0.3 µm.

7. A temper rolling mill according to Claim 6 which is a two stand mill.

8. A temper rolling mill according to Claim 6 or 7 wherein the scratch bright roll of the front stand has a surface roughness of at least 0.20 µm.

9. A temper rolling mill according to Claim 8 wherein the scratch bright roll of the front stand has a surface roughness of 0.5 to 1.0 µm.

10. A temper rolling mill according to any one of Claims 6 to 9 wherein the bright roll of the last stand is a mirror bright roll or a scratch bright roll.

## Patentansprüche

1. Nachwalzverfahren zum Nachwalzen eines Stahlblechs mit Hilfe eines Nachwalzwerks, das mit mehreren Walzgerüsten versehen ist, wobei mindestens die Walze am oberen vorderen Gerüst eine Riefenglanzwalze ist, die eine Oberflächenrauheit (Ra) von 1,2 µm oder weniger hat, und zumindest die Walze im letzten Gerüst eine Glanzwalze ist, die eine Oberflächenrauheit (Ra) von 0,5 µm oder weniger hat, **dadurch gekennzeichnet, dass** das Nachwalzen ein trockenes Walzen ist und dass das Stahlblech 0,012 Gewichtsprozent oder weniger an C enthält.

2. Nachwalzverfahren nach Anspruch 1, wobei das Nachwalzwerk ein Werk mit zwei Gerüsten ist.

3. Nachwalzverfahren nach Anspruch 1 oder 2, wobei das Stahlblech zwischen 0,001 und 0,008 Gewichtsprozent Kohlenstoff enthält.

4. Nachwalzverfahren nach Anspruch 1, 2 oder 3, wobei das Stahlblech zusätzlich zwischen 0,005 und 0,2 Gewichtsprozent Ti und/oder zwischen 0,002 und 0,1 Gewichtsprozent Nb enthält.

5. Nachwalzverfahren nach irgendeinem vorhergehenden Anspruch, wobei das Stahlblech zusätzlich nicht mehr als 0,15 Gewichtsprozent Al, nicht mehr als 0,2 Gewichtsprozent Si, zwischen 0,1 und 0,5 Gewichtsprozent Mn, nicht mehr als 0,05 Gewichtsprozent P und nicht mehr als 0,03 Gewichtsprozent S enthält.

6. Nachwalzwerk für Stahlblech, das mehrere Walzgerüste aufweist, wobei mindestens die Walze am oberen vorderen Gerüst eine Riefenglanzwalze ist, die eine Oberflächenrauheit (Ra) von 1,2 µm oder weniger hat, **dadurch gekennzeichnet, dass** zumindest die Walze im letzten Gerüst eine Glanzwalze ist, die eine Oberflächenrauheit (Ra) zwischen 0,15 und 0,3 µm hat.

7. Nachwalzwerk nach Anspruch 6, das ein Werk mit zwei Gerüsten ist.

8. Nachwalzwerk nach Anspruch 6 oder 7, wobei die Riefenglanzwalze des vorderen Gerüsts eine Oberflächenrauheit von mindestens 0,20 µm hat.

9. Nachwalzwerk nach Anspruch 8, wobei die Riefenglanzwalze des vorderen Gerüsts eine Oberflächenrauheit von 0,5 bis 1,0 µm hat.

10. Nachwalzwerk nach irgendeinem der Ansprüche 6 bis 9, wobei die Glanzwalze des letzten Gerüsts eine Hochglanzwalze oder eine Riefenglanzwalze ist.

## Revendications

1. Procédé d'écrouissage à froid pour l'écrouissage à froid d'une tôle d'acier, utilisant un laminoir d'écrouissage muni d'une pluralité de cages de laminage, dans lequel au moins le cylindre de laminoir de la cage à l'extrémité avant est un cylindre de laminoir à rayures brillant ayant une rugosité de surface (Ra) de 1.2 µm ou moins, et au moins un cylindre de laminoir de la dernière cage est un cylindre de laminoir brillant ayant une rugosité de surface (Ra) de 0.5 µm ou moins, **caractérisé en ce que** l'écrouissage à froid est un laminage à sec et **en ce que** la tôle d'acier contient 0.012% en poids ou moins de C.

2. Procédé d'écrouissage à froid selon la revendication 1, dans lequel le laminoir d'écrouissage est un laminoir à deux cages.

3. Procédé d'écrouissage à froid selon la revendication 1 ou 2, dans lequel la tôle d'acier contient de 0.001 à 0.008% en poids de carbone.

4. Procédé d'écrouissage à froid selon la revendication 1, 2 ou 3, dans lequel la tôle d'acier contient en outre de 0.005 à 0.2% en poids de Ti et/ou de 0.002 à 0.1% en poids de Nb.

5. Procédé d'écrouissage à froid selon l'une quelconque des revendications précédentes, dans lequel la tôle d'acier contient en outre pas plus de 0.15% en poids d'Al, pas plus de 0.2% en poids de Si, de 0.1 à 0.5% en poids de Mn, pas plus de 0.05% en poids de P, et pas plus de 0.03% en poids de S.

6. Laminoir d'écrouissage pour tôle d'acier ayant une pluralité de cages de laminage dans lequel au moins le cylindre de laminoir de la cage à l'extrémité avant est un cylindre de laminoir à rayures brillant ayant une rugosité de surface (Ra) de 1.2 µm ou moins, **caractérisé en ce que** le cylindre de laminoir de la dernière cage est un cylindre de laminoir brillant ayant une rugosité de surface (Ra) comprise entre 0.15 et 0.3 µm.

7. Laminoir d'écrouissage selon la revendication 6, qui est un laminoir à deux cages.

8. Laminoir d'écrouissage selon la revendication 6 ou 7, dans lequel le cylindre de laminoir à rayures brillant de la cage avant a une rugosité de surface d'au moins 0.20 µm.

9. Laminoir d'écrouissage selon la revendication 8, dans lequel le cylindre de laminoir à rayures brillant de la cage avant a une rugosité de surface comprise entre 0.5 et 1.0 µm.

10. Laminoir d'écrouissage selon l'une quelconque des revendications 6 à 9, dans lequel le cylindre de laminoir à rayures de la dernière cage est un cylindre de laminoir brillant de type miroir ou un cylindre de laminoir à rayures brillant.
